

April 9, 1968

H. TANCZYN

3,376,780

STAINLESS STEEL, PRODUCTS AND METHOD

Filed Sept. 19, 1966

3 Sheets-Sheet 1

FIG. 1



INVENTOR

Harry Tanczyn

BY

*John K. Tanczyn*

HIS ATTORNEY

April 9, 1968

H. TANCZYN

3,376,780

STAINLESS STEEL, PRODUCTS AND METHOD

Filed Sept. 19, 1966

3 Sheets-Sheet 1

FIG. 2



INVENTOR

Harry Tanczyn

BY

*John K. Kamm, Agent*

HIS ATTORNEY

April 9, 1968

H. TANCZYN

3,376,780

STAINLESS STEEL, PRODUCTS AND METHOD

Filed Sept. 19, 1966

3 Sheets-Sheet 3



FIG. 3

CHEMICAL ANALYSIS  
OF SPECIFIC EXAMPLE:

C .057%  
Mn 1.10%  
Si .50%  
Cr 16.02%  
Ni 8.07%  
Cu 3.20%  
Al 1.08%  
N .024%  
Fe Balance

HARDNESS - ROCKWELL "C"  
AT POINTS INDICATED.

INVENTOR

Harry Tanczyn

BY

*Joe H. Jant.*

HIS ATTORNEY

1

3,376,780

**STAINLESS STEEL, PRODUCTS AND METHOD**  
 Harry Tanczyn, Baltimore, Md., assignor to Armco  
 Steel Corporation, Middletown, Ohio, a corpora-  
 tion of Ohio

Continuation-in-part of application Ser. No. 249,506,  
 Jan. 4, 1963. This application Sept. 19, 1966, Ser.  
 No. 580,305

17 Claims. (Cl. 85—48)

**ABSTRACT OF THE DISCLOSURE**

Chromium-nickel-copper-aluminum stainless steel of such composition balance that in the annealed condition it is fully austenitic and readily lends itself to drastic cold-reduction and which, moreover, following cold-reduction, is readily hardened by ageing at moderate ageing temperatures. Such steel consists essentially of about 10% to 25% chromium-molybdenum with the actual chromium content being at least 10% and molybdenum up to 5% being substituted for chromium on a 1 to 1 basis; about 5% to 20% nickel-manganese with the actual nickel content being at least 4% and manganese up to 15% substituted for nickel on a 2 to 1 basis, with the relationship between the two groups being:

| Chromium-molybdenum,<br>percent: | Nickel-manganese,<br>percent |
|----------------------------------|------------------------------|
| 10                               | 13 to 20                     |
| 12                               | 8 to 20                      |
| 16                               | 7 to 20                      |
| 19                               | 6.5 to 20                    |
| 22                               | 5 to 20                      |
| 25                               | 5 to 20                      |

about 1% to 5% copper; about .25% to 2.50% aluminum; and remainder substantially all iron. In one specific embodiment the steel is of such particular composition balance that in the final age-hardened condition the metal remains austenitic and essentially non-magnetic. In a further embodiment the composition balance is such that the steel becomes magnetic in the age-hardened condition.

*Cross-reference to related application*

My application for patent is a continuation-in-part of my co-pending application Ser. No. 249,506 filed Jan. 4, 1963, now abandoned, and entitled Stainless Steel, Products and Method.

*Introduction*

The present invention is concerned with the austenitic chromium-nickel stainless steels, more particularly with such steels as are hardenable by heat-treatment. Concern also is with a method of hardening the same and with a variety of hardened articles and products fashioned of the steel.

One of the objects of my invention is the provision of a chromium-nickel stainless steel which works well in the mill as by rolling, drawing, and the like, in the production of sheet, strip, plate, bars, rods, wire and special shapes, which steel then is readily formed through cold-working operations such as drawing, upsetting, rolling, spinning and the like, as in the production of wire, springs, spun shapes and articles, rolled shapes and articles such as threaded fasteners having upset heads and rolled-on threads, all without necessity for intermediate annealing treatment; and which steel hardens to only a modest extent as a result of such cold-working or cold-forming operations and becomes susceptible to a subsequent age-hardening heat-treatment.

Another object is the provision of an austenitic chro-

2

mium-nickel stainless steel which is cold-formed easily into desired shapes with minimum wear on the forming equipment and which steel is then age-hardenable by heat-treatment at moderate temperatures and which in the work-hardened and age-hardened condition possesses the surprising combination of toughness and strength together with high surface hardness, abrasion-resistance and wear-ability.

A further object of my invention is the provision of a wide variety of radio antenna wire, instrument springs, industrial springs and the like, the provision of rolled shapes such as threaded fastening devices such as screws, bolts, etc., wherein the threaded portions thereof are rolled-on to give fastening devices which are tough, strong and present hard and abrasion-resistant threaded surfaces, which antenna wire, shapes, springs, fastening devices and the like are well adapted to withstand corrosion, wear and the stresses generally encountered in actual use.

An additional object is the provision of self-tapping screws, screws of such external or surface hardness and abrasion-resistance in the threaded portions thereof, and of such internal toughness and strength, as to serve in the tapping of metal parts such as sheet metal roofing, sidings and the like, and sheet metal housings for refrigerators, washing machines and other appliances, and then secure and fasten the same together.

Other objects of my invention in part will be obvious and in part particularly pointed to in the description which follows.

Accordingly, my invention resides in the combination of elements, in the mixture of ingredients and in the relation between the same, as well as in the various cold-working or cold-forming steps, in the various heat-treating steps and in the relation between composition, forming and heat-treatment, all as described herein, the scope of application of which is indicated in the claims at the end of this specification.

*Background of the invention*

As conducive to a better understanding of certain features of my invention, it may be noted at this point that the stainless steels have as of this date found great favor in the art. In all, there are available some 30-odd types, all suited to a number of different practical applications. Many of these are work-hardening, that is, they harden during cold-working and cold-forming operations. For example, the American Iron and Steel Institute Type 305 comprising about 18% chromium, 11% nickel, and remainder iron, has a relatively low work-hardening rate, but with a 60% reduction in area a hardness on the order of Rockwell C 50 may be obtained. Nevertheless, in any substantial working or forming operations intermediate and costly annealing treatments are required. Moreover, this steel cannot be significantly hardened by an ageing treatment.

The straight-chromium grades of stainless steel, for example Type 430, comprising about 17% chromium and remainder iron, as well as the Type 410 comprising about 12% chromium and remainder iron, although not inclined to harden as a result of cold-working operations, are not disposed to harden by ageing treatment either, that is, treatment at rather modest temperatures. Hardening of these steels is had by heating to high temperatures, that is, temperatures on the order of some 1800° F. and quenching, the high temperature causing scaling, which scaling must be removed at some expenditure of time and money. The structure is martensitic.

The more complex chromium-nickel stainless steels, for example, the chromium-nickel-copper-aluminum stainless steels made the subject of the Tanczyn U.S. Patent 2,694,626 of Nov. 16, 1954, although age-hardenable, are characterized by an objectionably high work-hardening rate.

This steel, like the others, is not suited to drastic cold-deformation and subsequent ageing to develop great hardness.

In the prior art self-tapping stainless steel screws are known. These customarily are made of the 12% chromium grade of stainless steel. The screws are hardened by heating at about 1800° F. and quenching. Following this they are relieved of quenching stresses by reheating at a temperature of about 400° F. to 600° F. The hardening treatment, however, leaves a heat-scale on the metal as noted above, with the result that the metal must be cleansed before use. Often to obtain a higher level of corrosion-resistance they are chromium-plated.

The self-tapping screws of the prior art are hardened throughout and for this reason are somewhat brittle.

One of the objects of my invention is the provision of a chromium-nickel-copper-aluminum stainless steel of such composition balance as to overcome the deficiencies of the steels of the prior art and be but moderately hardenable or greatly hardenable as desired, as a result of cold-deformation through cold-working and cold-forming operations; which cold worked or cold-formed steel then lends itself to age-hardening or precipitation-hardening by heat-treatment at moderate temperatures, i.e., temperatures not sufficiently high to cause formation of objectionable heat-scale; which steel and articles fashioned thereof are possessed of great surface hardness and abrasion-resistance, yet interiorly thereof are tough, ductile and adapted to withstand the stresses encountered in use; and which steel in the cold-worked and age-hardened condition is peculiarly adapted to withstand corrosive effects encountered in use, including those of galvanic origin.

#### *Summary of the invention*

Referring now more particularly to the practice of my invention, I provide a chromium-nickel-copper-aluminum stainless steel which consists essentially of a chromium-like metal in the amount of 10%-25%, a nickel-like metal in the amount of 5%-20%, copper in the amount of 1%-5%, aluminum in the amount of .25%-2.50%, with remainder substantially all iron. Now the chromium-like metal is chromium with or without the further ingredient molybdenum. In every instance the amount of chromium itself must be at least 10%. And the amount of molybdenum which may be included as a part of the chromium-like metal must not exceed 5%. Where molybdenum is employed along with chromium, replacement of molybdenum for chromium is on the basis of 1-1.

The nickel-like metal consists of nickel with or without the further ingredient manganese. The amount of nickel itself must be at least 4%. And where manganese is employed as a partial substitute for nickel, the substitution is on the basis of 2 for 1, with the total manganese content not exceeding 15%.

In the steel of my invention, carbon, of course, is present, this in amounts up to 0.20%, although I find that best results are had where the carbon content does not exceed 0.10%, particularly where it does not exceed 0.05%. Nitrogen also is present in small amounts, that is, amounts up to .25%, although here again, best result are achieved where the nitrogen content does not exceed 0.10%, and particularly where it does not exceed 0.05%.

In my steel the sum of the carbon and nitrogen contents ordinarily does not exceed 0.10%. Best results, as previously indicated, are had where both carbon and nitrogen are maintained at a minimum; particularly where the sum of the two does not exceed 0.05%, for I find that both of these ingredients increase the hardness of the steel in the annealed condition. And this necessitates additional working and forming to achieve a desired amount of plastic deformation. Any substantial carbon content, for example, carbon in excess of the 0.20% max. permissible figure, additionally would require objectionably high annealing temperatures in order to take the carbon into solution. And an excess of nitrogen additionally would run the

risk of gas evolution on freezing of the ingot with consequent unsoundness in the final product.

Silicon, likewise is present, this in amounts up to 2%. So, too, manganese in amounts up to 1% even where there is no purposeful manganese addition. Phosphorus and sulphur are present, each up to a maximum of about 0.05%.

The steel of my invention additionally may contain purposeful additions of boron in amounts up to 0.009% for improved hot-working properties in the presence of the high total alloy content. Titanium, zirconium and columbium also may be included where desired in amounts up to about 1%, to obtain an improvement in age-hardenability. These additions have no significant effect on work-hardening. The ingredients selenium, lead, bismuth, tellurium and silver, as well as phosphorus and sulphur, may be present in sum total up to 0.50% as a maximum, to lend improved machinability to the metal where required in certain applications. These additions are not included in the steel of my invention where cold-heading operations or other cold-upsetting operations are resorted to, or where significant bending stresses are contemplated. In general, my steel is free of these additions.

#### *Brief description of the drawings*

In the accompanying drawings:

FIGURE 1 presents in graphic form the tensile properties of wire according to my invention which has been annealed and then cold-drawn differing amounts and wire which, subsequent to the cold drawing has been age-hardened,

FIGURE 2 illustrates the hardness of the wire of FIGURE 1 for differing cold-reductions, and

FIGURE 3 illustrates on greatly enlarged scale, a ground and polished section of a self-tapping Phillips head screw according to my invention.

#### *Description of the preferred embodiments*

Now in the steel of my invention I employ a particular balance or relationship between the chromium-like component, on the one hand, and the nickel-like component, on the other. I find that where there is a high ratio between the chromium-like content and the nickel-like content, substantially uniform elongation is achieved in working, but that the work-hardening rate is unduly high; such a steel has a high work-hardening factor.<sup>1</sup> Where, however, the ratio between the chromium-like and the nickel-like ingredients is low, that is, less than 1, the elongation of the metal is not uniform; it tends to neck down. And even though the rate of work-hardening is acceptable, the steel is not satisfactory.

In the steel of my invention the work-hardening factor amounts to about 85, this falling well below the 162 work-hardening factor of the Type 301 steel (17% chromium, 7% nickel, and remainder iron), a steel of objectionably high work-hardening rate. It falls very close to the very low work-hardening factor of 80 which is had in a 16-18 steel (16% chromium, 18% nickel, and remainder iron). This latter steel, however, is subject to objectionable localized elongation.

While the balance between the chromium-like and the nickel-like components of my steel is generally such that the steel in the annealed condition is non-magnetic, a balance substantially exceeding 2 is inclined to give a duplex structure, wherein the metal does not work well in the hot mill. It is inclined to break and tear through the ferrite constituent.

Now in the cold-worked and age-hardened condition my steel may become magnetic or it may remain non-magnetic, depending upon the particular balance of ingredients. For the magnetic steel I employ a nickel-like content of about 13% to 16% for a chromium-like con-

<sup>1</sup> "The Cold-Work-Hardening Properties of Stainless Steel in Compression" by Bloom, Goller and Mabus: 1947 Transactions A.S.M., volume 39, page 843.

tent of 10%, a nickel-like content of 8%-14% for a chromium-like content of about 12%, a nickel-like content of 7%-13% for a chromium-like content of 16%, a nickel-like content of 6.5%-9.5% for a chromium-like content of 19%, and a nickel-like content of 5%-6% for a chromium-like content of 22%. In these steels the copper content amounts to about 3% and the aluminum content about 1%, although in general some latitude is desirable; the copper ranging from 3%-4%, permissibly from 1%-5%, and the aluminum from .75%-1.50%, although permissible from .25% to 2.50%.

While all the above steels are essentially austenitic in the annealed condition, the steel of 22% chromium content does contain some ferrite. But when subjected to drastic cold-deformation all of the steels become martensitic and magnetic. This condition obtains even in the steel of 10% chromium content with a nickel content of 13% to 16% where the cold-deformation amounts to as much as 70%. These steels, of course, remain martensitic and magnetic even after a subsequent age-hardening treatment.

In the magnetic steels manganese may be partially substituted for nickel, this on a 2 to 1 basis, as noted above. Where the chromium content of the particular steel is below 16%, the manganese content may be as much as 12%, this being substituted for 6% nickel. But where the chromium content is above 16%, no more than about 8% manganese may be employed, this as a substitute for 4% nickel. In these steels it will be understood, as previously indicated, that the actual nickel content must be at least 4% in order to enjoy the desired combination of work-hardening and age-hardening properties.

Now in the non-magnetic steel, i.e. the steel which is non-magnetic in the annealed condition, non-magnetic in the work-hardened condition and non-magnetic in the age-hardened condition, I employ a nickel-like content of 15%-20% for a chromium-like content of 10%, a nickel-like content of 14%-20% for a chromium-like content of 12%, a nickel-like content of 12%-20% for a chromium-like content of 16%, a nickel-like content of 11%-20% for a chromium-like content of 19%, a nickel-like content of 14%-20% for a chromium-like content of 22%, and a nickel-like content of 15%-20% for a chromium-like content of 25%. In each of these steels the copper content amounts to about 3% and the aluminum content about 1%, although the copper may range from about 1%-5%, preferably 2%-4%, and the aluminum from .25%-2.50%, preferably .75%-1.50%.

In the non-magnetic steel manganese may be partially substituted for nickel up to about 15% of manganese, this for 7.5% nickel. The actual nickel content, as previously indicated, must be at least 4%.

In the steel of my invention the amounts of the ingredients chromium, nickel, copper and aluminum, as well as the amounts of the ingredients molybdenum, and manganese, which were partially substituted for chromium, and nickel, respectively, are in every sense critical. So, too, is the relation between the several ingredients. As noted above, the chromium-like component ranges from 10% to 25%, with the actual chromium content being at least 10%. Where the actual chromium content is less than the 10% figure, and more particularly where it is less than 12%, the required corrosion-resistant qualities are not had. And where the chromium-like component exceeds the 25% figure, I find that the nickel requirements necessary become excessive in order to achieve the combination of work-hardening and age-hardening. The chromium content of my steel preferably ranges from 14%-19%.

While the molybdenum content of my steel may range up to 5% as a partial substitute for chromium, an amount in excess of the 5% figure is not acceptable because excessive hardening is had, with loss of cold-working properties.

Now the nickel-like component, as noted above, ranges from about 5%-20%. The actual nickel content, however, where manganese is partially substituted for nickel, may not be less than 4% for otherwise, the steel becomes unstably austenitic and the desired combination of work-hardening and age-hardening is not had. The manganese substituent may not exceed 15%; actually, it may not exceed 12% for the magnetic steels of chromium contents below 16% and may not exceed 8% for the steels of chromium content above 16%, as previously noted, for I find that higher manganese contents as well as higher nickel contents disturb the composition balance necessary to achieve the combination of initial work-hardening and subsequent age-hardening treatments.

In the steels of my invention both copper and aluminum serve to lower the work-hardening rate, that is, lower it to an acceptable figure. The copper content, while permissibly ranging from 1%-5%, preferably does not exceed 4% because I find that amounts significantly above the 4% figure are inclined to adversely affect the hot-rolling properties of the metal; apparently the limit of solubility for copper is about 4%, and any excess appears as free copper, introducing a liquid phase with resulting breaking in the mill unless the hot-rolling operation is conducted at an undesirably lowered temperature. A copper content below the 1% figure has no beneficial effect; excessive amounts of aluminum would be required and this, in turn, would require an excessive amount of nickel, for the reason that aluminum apparently lowers the activity of the nickel present in the steel. Best results are had with a copper content of 2%-4%, as previously noted.

The aluminum content of my steel permissibly ranges from .25%-2.50%. Below the .25% figure there is no beneficial effect, and above a figure of 2.50%, the nickel requirement again becomes excessive. I find that best results are had where the aluminum content ranges from about .75% to 1.50%.

The steel of my invention conveniently is melted in the electric arc furnace or by other means known to those skilled in the art to which the invention relates. On this further comment is believed unnecessary, save to remark that the steel handles well in the furnace, tems well and the ingot mold strips from the ingot with ease.

Ingots, blooms, billets, and the like, work well in the hot mill at conventional rolling temperatures, as in the production of plate, sheet, strip, bars, rods, wire, and special shapes. The hardness of the metal in the hot-rolled condition and in the annealed condition is on the order of Rockwell B 60-80. And upon cleaning, it is suited to a variety of cold-working and cold-forming operations, such as upsetting, rolling, drawing, spinning, and the like, in the production of screws, bolts and other headed and threaded fasteners, instrument springs and industrial springs, washers, and various machine parts.

In the cold-working and cold-forming operations the steel of my invention acquires significant hardness; the hardness customarily increases up to about Rockwell C 37 for the steels of such composition balance as to be martensitic and magnetic, and up to about Rc 26 for the steels which are of such composition balance as to be fully austenitic and non-magnetic. These maximum hardness figures represent cold-reductions on the order of some 60%-70%. Even greater hardnesses are had where drastic cold-reductions are employed, that is, reductions approaching 90% as more particularly discussed herein-after. It will be seen that in the martensitic and magnetic steels such hardnesses amount to some Rockwell C 46 for a reduction of 87%.

Following the cold-working and cold forming operation the steel is age-hardened, the ageing temperature employed being dependent upon the composition. For the steel and articles of magnetic composition balance, for example, 15%-18% chromium, 7%-10% nickel, 2%-5% copper, .75%-1.50% aluminum, and remainder substantially all iron, hardening is achieved by heating the

same at a temperature of about 700° F.-900° F. and cooling in any one of air, oil or water. I find that the cold-working operation has sufficiently strained the metal to induce age-hardening by the comparatively low-temperature ageing treatment. My steel and articles are free of

the chemical analyses of several specific examples are given in Table I below; those being martensitic and magnetic in the final age-hardened condition are given under I(a) and those remaining austenitic and non-magnetic in the aged condition are given under I(b):

TABLE I.—CHEMICAL ANALYSES OF TYPICAL CR-NI-CU-AL STAINLESS STEELS OF THE INVENTION  
[I(a) Magnetic as age-hardened]

| Heat No.                            | C    | Mn   | Si  | Cr    | Ni    | Cu   | Al   | N    | Mo   |
|-------------------------------------|------|------|-----|-------|-------|------|------|------|------|
| R3609                               | .069 | .38  | .60 | 16.04 | 7.09  | 2.02 | 1.12 | —    | —    |
| R3615                               | .063 | .40  | .59 | 15.97 | 7.11  | 2.96 | 1.03 | —    | —    |
| R3682                               | .070 | .36  | .44 | 15.06 | 8.08  | 3.05 | .87  | —    | —    |
| R3685                               | .074 | .38  | .54 | 14.17 | 9.17  | 3.02 | .80  | —    | —    |
| R3472                               | .080 | 1.02 | .51 | 15.95 | 7.08  | 3.00 | 1.13 | .026 | —    |
| R3638                               | .067 | 1.10 | .63 | 17.18 | 8.17  | 2.98 | .53  | —    | —    |
| R3728                               | .076 | 1.04 | .37 | 16.32 | 8.24  | 2.82 | .59  | .029 | —    |
| R3729                               | .078 | 1.05 | .41 | 16.01 | 9.15  | 2.94 | .77  | —    | —    |
| R3814                               | .083 | .94  | .55 | 16.54 | 8.00  | 2.89 | 1.16 | —    | —    |
| R3919                               | .067 | 1.10 | .50 | 16.02 | 8.07  | 3.20 | 1.03 | .024 | —    |
| High Manganese Variation            |      |      |     |       |       |      |      |      |      |
| R3473                               | .077 | 2.94 | .59 | 15.16 | 7.07  | 2.94 | 1.18 | .027 | —    |
| Low Carbon Variation                |      |      |     |       |       |      |      |      |      |
| R3960                               | .024 | 1.01 | .37 | 16.16 | 9.11  | 3.40 | 1.16 | —    | —    |
| R3970                               | .015 | 1.17 | .45 | 16.09 | 8.10  | 3.38 | 1.06 | .026 | —    |
| Molybdenum Variation                |      |      |     |       |       |      |      |      |      |
| R3893                               | .072 | 1.03 | .47 | 14.02 | 8.14  | 2.89 | 1.17 | —    | 1.98 |
| R3894                               | .074 | .96  | .38 | 12.56 | 8.16  | 2.90 | 1.20 | —    | 4.06 |
| [I(b) Non-magnetic as age-hardened] |      |      |     |       |       |      |      |      |      |
| R3630                               | .059 | 1.06 | .60 | 17.33 | 10.24 | 2.98 | .54  | .027 | —    |
| R3640                               | .073 | 1.06 | .57 | 16.86 | 12.10 | 2.97 | .55  | —    | —    |
| R3641                               | .070 | 1.13 | .61 | 17.33 | 14.2  | 2.97 | .67  | —    | —    |
| R3644                               | .084 | 1.23 | .76 | 16.58 | 16.25 | 2.94 | 2.44 | .026 | —    |
| R3653                               | .060 | 1.05 | .49 | 12.63 | 15.14 | 2.97 | .75  | —    | —    |
| R3730                               | .070 | 1.04 | .42 | 16.18 | 10.21 | 2.93 | .75  | —    | —    |
| R3801                               | .065 | 1.07 | .48 | 15.36 | 14.32 | 3.02 | 1.50 | —    | —    |
| R3804                               | .055 | .90  | .32 | 14.12 | 14.48 | 2.98 | 1.68 | —    | —    |

scale, or other objectionable surface effect. In the aged condition the hardness had amounts up to about Rockwell C 52 for reductions on the order of 60% and up to about Rockwell C 57 for reductions approaching 90%.

Similarly, for the steel and articles of such composition balance as to be fully austenitic in the aged condition and free of magnetic effects, that is, the steel analyzing about 15%-18% chromium, 11% to 13% nickel, 2% to 5% copper, .75%-1.50% aluminum, and remainder substantially all iron, ageing is achieved by heating the metal at a temperature of about 1050° F.-1250° F. and then

35 The hardness of the steels of Table I in the annealed condition, as well as the work-hardening factor for the same, the hardness had when reduced 40% and when reduced 60%, and the final hardness in the age-hardened condition both for the 40% reduced steels and the 60% reduced steels are given in Table II below. Here again 40 the steels which are magnetic in the age-hardened condition are given under II(a) and those remaining non-magnetic after ageing are given under II(b). In each instance the hardness data was developed on wire of analysis specified initially of  $\frac{3}{8}$ " diameter by 15" length.

TABLE II.—HARDNESS AND WORK-HARDENING FACTORS OF THE CRNI-CU-AL STAINLESS STEELS OF TABLE I  
II(a) Magnetic as Age-Hardened<sup>1</sup>

| Heat No.                                          | Cold Work Hardening Factor | Annealed <sup>2</sup> Hardness Rockwell | Cold Drawn 40% Hard. Rockwell | Cold Drawn 60% Hard. Rockwell | Cold drawn 40% and Aged Rockwell | Cold Drawn 60% and Aged Rockwell |
|---------------------------------------------------|----------------------------|-----------------------------------------|-------------------------------|-------------------------------|----------------------------------|----------------------------------|
| R3609                                             |                            | B82                                     | C34                           | C44                           | C48                              | C53                              |
| R3615                                             |                            | B66                                     | C29                           | C42                           | C43                              | C51                              |
| R3682                                             | 109.5                      | B76                                     | C31                           | C35                           | C39                              | C50                              |
| R3685                                             | 100.8                      | B78                                     | C31                           | C35                           | C39                              | C42                              |
| R3472                                             | 85.7                       | B75                                     | C32                           | C36                           | C47                              | C51                              |
| R3638                                             | 87.7                       | B79                                     | —                             | —                             | —                                | —                                |
| R3728                                             | 91.8                       | B78                                     | C29                           | C36                           | C34                              | C46                              |
| R3729                                             | 85.4                       | B80                                     | C24                           | —                             | C31                              | —                                |
| R3814                                             | 92.9                       | B80                                     | C30                           | C36                           | C33                              | C41                              |
| R3919                                             | 86.3                       | B68                                     | C31                           | C36                           | C44                              | C48                              |
| High Manganese Variation                          |                            |                                         |                               |                               |                                  |                                  |
| R3473                                             | 84.7                       | B75                                     | C26                           | C35                           | C36                              | C48                              |
| Low Carbon Variation                              |                            |                                         |                               |                               |                                  |                                  |
| R3960                                             | 80.2                       | B63                                     | C23                           | C30                           | C29                              | C40                              |
| R3970                                             | 81.8                       | B65                                     | C26                           | C36                           | C40                              | C49                              |
| Molybdenum Variation                              |                            |                                         |                               |                               |                                  |                                  |
| R3893                                             | 102.2                      | B78                                     | C31                           | C36                           | C37                              | C48                              |
| R3894                                             | 104.5                      | B80                                     | C31                           | C35                           | C36                              | C48                              |
| [II(b) Non-magnetic as age-hardened] <sup>3</sup> |                            |                                         |                               |                               |                                  |                                  |
| R3644                                             | 78.5                       | B72                                     | C24                           | C28                           | C37                              | C41                              |
| R3801                                             | 77.1                       | B73                                     | C26                           | C30                           | C35                              | C38                              |
| R3804                                             | 79.0                       | B72                                     | C25                           | C31                           | C35                              | C39                              |

<sup>1</sup> Anneal, 850° F. for 1 hr. and air-cool. <sup>2</sup> Anneal 1,900° to 1,950° F., 20 min., water-quench. <sup>3</sup> Anneal, 1,100° F. for 5 hrs. and air-cool.

quenching in air, oil or water. The hardness had there comes up to about Rockwell C 40 for reductions of about 60% and a hardness of about Rockwell C 44 for a reduction approaching 90%.

As generally illustrative of the steels of my invention,

75 It will be seen from the test data presented above that in the annealed condition both the magnetic and non-magnetic steels of my invention have a hardness on the order of Rockwell B 63-82. No particular difference in hardness between the two steels is apparent in either the

annealed condition or in the hot-rolled condition. In the cold-worked condition, however, the martensitic and magnetic steel with about 40% reduction, had a hardness of some Rockwell C 23-34 and with a 60% cold-

proaching 90%) and in the cold-drawn and age-hardened condition. The chemical composition of the specific example and the mechanical properties are reported in Table III below:

TABLE III.—CHEMICAL COMPOSITION AND MECHANICAL PROPERTIES OF ANNEALED, COLD-DRAWN AND COLD-DRAWN-AGE-HARDENED WIRE SECTIONS

| Heat No.              | C                 | Mn                                    | P                                      | S              | Si                   | Cr                   | Ni   | Cu   | Al   |
|-----------------------|-------------------|---------------------------------------|----------------------------------------|----------------|----------------------|----------------------|------|------|------|
| 034067.....           | 0.050             | .65                                   | .012                                   | .012           | .50                  | 15.25                | 7.47 | 3.14 | 1.92 |
| Wire Dia.<br>(inches) | Condition         | Ult.Tens Str.,<br>p.s.i. <sup>2</sup> | 0.2% Yld. Str.,<br>p.s.i. <sup>2</sup> | Percent Elong. | Percent Red.<br>Area | Rockwell<br>Hardness |      |      |      |
| .253                  | Annealed.....     | 89/92                                 | 26/28                                  | 46/47          | 65/66                | B68                  |      |      |      |
| .245                  | CD 5%+H-900.....  | 103/103                               | 62/62                                  | 43/40          | 67/68                | B80                  |      |      |      |
| .245                  | CD 5%+H-900.....  | 99/100                                | 62/68                                  | 41/41          | 67/67                | B81                  |      |      |      |
| .237                  | CD 10%.....       | 109/110                               | 71/74                                  | 33/37          | 62/63                | B96                  |      |      |      |
| .237                  | CD 10%+H-900..... | 105/106                               | 80/81                                  | 33/37          | 65/66                | B98                  |      |      |      |
| .224                  | CD 20%.....       | 122/123                               | 75/78                                  | 32/33          | 61/61                | C23                  |      |      |      |
| .224                  | CD 20%+H-900..... | 125/126                               | 109/109                                | 33/34          | 60/61                | C24                  |      |      |      |
| .194                  | CD 40%.....       | 140/140                               | 110/111                                | 24/18          | 59/61                | C28                  |      |      |      |
| .194                  | CD 40%+H-900..... | 165/165                               | 141/141                                | 18/18          | 59/59                | C35                  |      |      |      |
| .158                  | CD 60%.....       | 170/172                               | 162/168                                | 14/14          | 56/56                | C35                  |      |      |      |
| .158                  | CD 60%+H-900..... | 234/235                               | 200/204                                | 14/14          | 51/51                | C46                  |      |      |      |
| .137                  | CE 70%.....       | 189/190                               | 180/182                                | 13/15          | 52/53                | C39                  |      |      |      |
| .137                  | CD 70%+H-900..... | 284/288                               | 250/255                                | 11/12          | 47/48                | C51                  |      |      |      |
| .112                  | CD 80%.....       | 217/222                               | 209/219                                | 11/11          | 49/49                | C44                  |      |      |      |
| .112                  | CD 80%+H-900..... | 310/314                               | 279/284                                | 11/11          | 40/43                | C56                  |      |      |      |
| .100                  | CD 84%.....       | 229/233                               | 204/210                                | 10/10          | 41/47                | C45                  |      |      |      |
| .100                  | CD 84%+H-900..... | 328/330                               | ( <sup>3</sup> )                       | 9/10           | 40/42                | C57                  |      |      |      |
| .090                  | CD 87%.....       | 235/238                               | 210/215                                | 6/9            | 41/41                | C46                  |      |      |      |
| .090                  | CD 87%+H-900..... | 335/336                               | ( <sup>3</sup> )                       | 11/11          | 40/40                | C57                  |      |      |      |

<sup>1</sup> Aluminum content checked 4" billet section, H-900=900° F., 1 hr., —air cool.

<sup>2</sup> P.s.i.  $\times$  1,000.

<sup>3</sup> No offset shown.

reduction, a hardness of Rc 30-44. The austenitic and non-magnetic steel when subjected to a reduction of 60% has a hardness of Rc 28-31 for the examples given.

When aged, following work-hardening, the martensitic and magnetic steels (heating at 850° F. and air-cooled) have a hardness of some Rockwell C 29-48 for the steels with 40% cold-reduction and a hardness of some Rc 40-53 for those with 60% cold-reduction. The non-magnetic steels when aged (1100° F. and air-cooled) following the 40% cold-reduction, have a hardness of some Rc 35-37 for the examples given, and following the 60% cold-reduction have a hardness of Rc 34-41. Greatest hardening is had with the magnetic or martensitic steels.

As more particularly illustrated of the great strength had in the martensitic and magnetic steels of my invention when cold-drawn up to about 90% reduction, a specific example in the form of wire analyzing about 15% chromium, about 7%-8% nickel, about 3% copper, about 1% aluminum, and remainder substantially all iron, was tested in the annealed condition, in the cold-drawn condition (for various amounts of drawn ap-

45 The ultimate tensile strength, the percentage elongation in 2" and the percentage reduction in area for the examples of cold-drawn, and cold-drawn and age-hardened steel wire of Table III, are graphically illustrated in FIGURE 1 of the accompanying drawings for differing percentages of cold reduction. The hardnesses had for the differing cold-reductions is illustrated in the FIGURE 2. It is to be especially noted that while there is an increase in tensile strength and hardness with an increase in the cold reductions, the ductility of the metal, as exemplified by the reduction of area and the elongation figures, is well retained. These fall but little until reductions of 70% or especially reductions of 80% and more are made. It is the subsequent age-hardening treatment, however, which imparts the great strength and hardness which 30 35 characterize the steel.

40 Note that with the age-hardening treatment these severely cold-reduced steels enjoy an increase in tensile strength of some 90,000 to 100,000 p.s.i. to reach tensile strengths exceeding 300,000 p.s.i. for the more severely reduced steels (from about 190,000 to 285,000 p.s.i., an

TABLE IV.—HARDNESS AND ROOM TEMPERATURE TENSILE PROPERTIES OF NON-MAGNETIC PRECIPITATION-HARDENABLE STAINLESS STEELS

| Heat No.                                              | C        | Mn                      | Si                     | Cr             | Ni                | Cu   | Al   | N     |
|-------------------------------------------------------|----------|-------------------------|------------------------|----------------|-------------------|------|------|-------|
| R3644.....                                            | .084     | 1.23                    | .76                    | 16.58          | 16.25             | 2.94 | 2.44 | .026  |
| R3801.....                                            | .065     | 1.07                    | .48                    | 15.36          | 14.32             | 3.02 | 1.50 | ..... |
| R3804.....                                            | .055     | .90                     | .32                    | 14.12          | 14.48             | 2.98 | 1.68 | ..... |
| Condition                                             | Heat No. | Ult. Tens. Str., p.s.i. | 0.2% Yld. Str., p.s.i. | Percent Elong. | Rockwell Hardness |      |      |       |
| Annealed, 1925° F., 20 mins. water quench.            | R3644    | 74,000                  | 29,000                 | 56             | B72               |      |      |       |
|                                                       | R3801    | 76,000                  | 28,700                 | 57             | B73               |      |      |       |
|                                                       | R3804    | 74,500                  | 28,500                 | 57             | B72               |      |      |       |
| Annealed plus cold-drawn 40%.....                     | R3644    | 132,000                 | 98,000                 | 40             | C24               |      |      |       |
|                                                       | R3801    | 134,000                 | 101,000                | 41             | C26               |      |      |       |
|                                                       | R3804    | 135,000                 | 99,000                 | 39             | C25               |      |      |       |
| Annealed, cold-drawn 40%+1,100° F., 5 hrs., air cool. | R3644    | 165,000                 | 138,000                | 28             | C37               |      |      |       |
|                                                       | R3801    | 161,000                 | 130,000                | 31             | C35               |      |      |       |
|                                                       | R3804    | 159,000                 | 125,000                | 32             | C35               |      |      |       |
| Annealed, cold-drawn 60%.....                         | R3644    | 145,000                 | 120,000                | 32             | C28               |      |      |       |
|                                                       | R3801    | 147,000                 | 115,000                | 30             | R30               |      |      |       |
|                                                       | R3804    | 148,000                 | 119,000                | 31             | R31               |      |      |       |
| Annealed, cold-drawn 60%+1,100° F., 5 hrs., air cool. | R3644    | 178,000                 | 147,000                | 21             | C41               |      |      |       |
|                                                       | R3801    | 170,000                 | 140,000                | 23             | C38               |      |      |       |
|                                                       | R3804    | 172,000                 | 145,000                | 20             | C39               |      |      |       |
| Annealed, cold-drawn 80%.....                         | R3644    | 170,000                 | 150,000                | 22             | C37               |      |      |       |
|                                                       | R3801    | 171,000                 | 158,000                | 20             | C38               |      |      |       |
|                                                       | R3804    | 168,000                 | 159,000                | 20             | C38               |      |      |       |
| Annealed, cold-drawn 80%+1,100° F., 5 hrs., air cool. | R3644    | 197,000                 | 183,000                | 17             | C44               |      |      |       |
|                                                       | R3801    | 195,000                 | 180,000                | 16             | C42               |      |      |       |
|                                                       | R3804    | 192,000                 | 178,000                | 18             | C43               |      |      |       |
| Annealed, cold-drawn 90%.....                         | R3644    | 179,000                 | 165,000                | 18             | C39               |      |      |       |
|                                                       | R3801    | 181,000                 | 167,000                | 17             | C40               |      |      |       |
|                                                       | R3804    | 182,000                 | 169,000                | 17             | C41               |      |      |       |
| Annealed, cold-drawn 90%+1,100° F., 5 hrs., air cool. | R3644    | 205,000                 | 191,000                | 15             | C45               |      |      |       |
|                                                       | R3801    | 198,000                 | 186,000                | 14             | C44               |      |      |       |
|                                                       | R3804    | 195,000                 | 187,000                | 14             | C44               |      |      |       |

increase of 95,000 p.s.i., for the 70% cold-reduced steel; from about 220,000 to about 310,000 p.s.i., an increase of 90,000 p.s.i., for the 80% cold-reduced steel; and from about 235,000 to 335,000 p.s.i., an increase of 100,000 p.s.i., for the 87% cold-reduced steel). Yet the great hardness and strength of the severely cold drawn wire (some Rockwell C 57 and a tensile strength of 335,000 p.s.i. for the 87% cold-drawn and aged sample of Table III) are had without sacrifice of ductility, the elongation amounting to some 11% and the reduction in area being some 40%; there is little change in the elongation and reduction in area figures as a result of the ageing treatment. The combination of great strength and hardness along with good retained ductility permits the drastically cold-reduced and age-hardened steel wire to be wound into a variety of springs.

Samples of three non-magnetic stainless steels were cold-drawn from  $\frac{3}{8}$ " diameter wire in differing amounts up to 90% and then age-hardened. The chemical composition of these steels and their mechanical properties in the cold-drawn and in the cold-drawn and age-hardened condition are given in Table IV.

It is to be noted that the drastically cold-reduced samples of 80% and 90% reductions in the annealed conditions have tensile strengths of some 168,000-171,000 p.s.i. for the 80% reductions and some 179,000-182,000 p.s.i. for the 90% reductions. In the age-hardened condition these strengths rise to some 192,000-197,000 p.s.i. for the lesser reductions and to some 195,000-205,000 p.s.i. for the greater reductions. The increase in strength with the ageing treatment amounts to some 24,000-27,000 p.s.i. for the 80% reductions and some 13,000-26,000 p.s.i. for those reduced 90%. The ductility of the steel, as reflected by the elongation figures, is well retained with the ageing treatment, the elongation falling only from 20-22% down to 16-18% for the samples reduced 80% and only from 17-18% down to 14-15% for those reduced 90%.

In the work-hardened and age-hardened condition, the steels of my invention possess a combination of high surface or external hardness together with internal toughness and ductility; the internal hardness is substantially lower than the surface hardness. And of particular consequence, the hardness of the finished metal is greatest at the points where the greatest cold-working has been had and least where the least amount of cold-working results. In every case, however, the final hardness achieved is not that of the cold-working operation, but it is that of the combination of cold-working and age-hardening. Particularly great strength in combination with significant ductility is had with the martensitic steels reduced in the amount of some 70%-90% and especially about 80%-90%. Note that with the age-hardening these severely cold-reduced steels enjoy an increase in tensile strength of some 90,000 to 100,000 p.s.i. as a result of the ageing treatment to reach tensile strengths exceeding 300,000 p.s.i. for the more severely reduced steels (from 190,000 to 285,000 p.s.i., an increase of 95,000 p.s.i., for the 70% cold-reduced steel; from 220,000 to 310,000 p.s.i., an increase of 90,000 p.s.i., for the 80% cold-reduced steel; and from 235,000 to 335,000 p.s.i., an increase of 100,000 p.s.i., for the 87% cold-reduced steel). And it is noted even the most severely cold-reduced steel, following the age-hardening treatment, enjoys substantial ductility, this on the order of 11% elongation in 2" and a reduction in area of about 40%.

As particularly illustrative of the practice of my invention, reference is made to the production of self-tapping drive screws, this by way of automatic machinery, the screws being produced at the rate of about 300 a minute. In this operation wire stock, typically 0.132" diameter, is upset in forming the screw head. The head then may be provided with a milled slot or it may be recessed to provide a Phillips head. The required thread is rolled on. In this cold-rolling operation, as well as in the cold-

upsetting operation, the extent of the cold-reduction had approaches 60% or more. The resulting hardness comes to Rockwell C 37, although it only may amount to some Rockwell C 26, depending upon the composition balance, that is, whether such as to give magnetic or non-magnetic screws.

The cold-formed screws are subjected to age-hardening treatment with a resultant increase in hardness approaching Rockwell C 52 for the screws with a cold-worked hardness approaching Rockwell C 37 (magnetic, with ageing at 700°-900° F.) and a hardness approaching Rockwell C 40 for those having a cold-work hardness approaching Rockwell C 26 (non-magnetic, with ageing at 1050°-1250° F.).

All of the screws in the age-hardened condition are possessed of a surprising combination of great surface hardness, particularly at the extreme edges of the threads, together with much reduced hardness and great toughness and ductility throughout the core of the screw. The surface of the sunken head likewise is hard and is admirably adapted to accommodate a driving tool, that is, power screwdriver or manual screwdriver. The threads of high surface hardness are abrasion-resistant and cut into metal siding, sheathing, and the like, as a self-tapping operation. And the screws are well suited to secure metal pieces together, holding them firmly without thread breakage.

Screws of the particular composition balance resulting in an austenitic and non-magnetic structure are peculiarly adapted to the securing of aluminum siding, roofing, and the like, as well as refrigerator, washing-machine and other aluminum housings, in that they are free of the hydrogen-embrittling effect resulting from galvanic action found in certain screws of the prior art, notably those of martensitic structure.

With regard to the self-tapping drive screw of my invention, attention is directed to the FIGURE 3 of the accompanying drawing showing, on much enlarged scale, one-half of a Phillips screw, the other half of which has been removed by grinding operation, the screw being fashioned of .132" diameter wire of the Heat R3919 of chemical analysis reported in Table I above and aged at 850° F. for 5 hours and air-cooled following fabrication. Hardness determinations made along the central core of the screw as well as those made along the roots of the threads and the extreme tips of the threads are given in Rockwell C figures. So, too, the hardness had along the head of the screw is given. It is noted that while the core of the screw has a hardness of some Rockwell C 22-25 (the hardness determinations were made at the particular points indicated adjacent the hardness numbers), the hardness along the root of the threads amounts to some Rockwell C 30-39. Further along the threads the hardening is about Rc 39-42. At the extreme outer edges of the threads the hardness is some Rc 50-52. The tip of the screw has a hardness of about Rc 47 and the head is seen to have a hardness of some Rc 35-39 except at the recess. There the hardness amounts to Rc 42-46. On the basis of hardness tests made on cold-drawn and aged sections of wire for Heat R3919 it is estimated that local reduction in area on the self-tapping screw ranges up to 70%, this at the extreme outer edges of the threads.

The self-tapping screw of my invention is well suited to tapping and then securing of sheet metal sections of iron, aluminum, copper, brass and the like, the particular composition balance being selected to avoid galvanic effects in connection with aluminum sections. The screws for aluminum sections preferably are fully austenitic and non-magnetic. The austenitic, and non-magnetic, steel also is suited to the production of instrument springs, instrument panels, dials, pointers and the like.

As further illustrative of the practice of my invention reference is made to the manufacture of radio antenna wire. The chemical composition of the wire, the sequence of operational steps employed (for Hot-rolled and then Cold-drawn, Line-Up No. 1 and for Annealed and Cold-

Drawn, Line-up No. 2) and the resulting mechanical properties are given in Table V below:

and manganese, with an actual nickel content of at least 4% and manganese up to 15% being substituted for nickel

TABLE V.—MANUFACTURE OF .200" DIAMETER RADIO ANTENNA WIRE FROM  $\frac{3}{8}$ " HOT-ROLLED WIRE<sup>1</sup>

| Condition                                                                    | Lineup No. 1                   |                                 |                   |                 | Lineup No. 2                   |                                 |                   |                 |
|------------------------------------------------------------------------------|--------------------------------|---------------------------------|-------------------|-----------------|--------------------------------|---------------------------------|-------------------|-----------------|
|                                                                              | U.T.S.,<br>p.s.i. <sup>2</sup> | 0.2% YS,<br>p.s.i. <sup>2</sup> | Percent<br>Elong. | Percent<br>R.A. | U.T.S.,<br>p.s.i. <sup>2</sup> | 0.2% YS,<br>p.s.i. <sup>2</sup> | Percent<br>Elong. | Percent<br>R.A. |
| Hot-rolled $\frac{3}{8}$ " Rd.                                               | 98/102                         | 48/55                           | 45/46             | 53/59           | 88/90                          | 26/28                           | 45/50             | 67/68           |
| Annealed                                                                     |                                |                                 |                   |                 |                                |                                 |                   |                 |
| CD 70%, .206" Rd.                                                            | 212/213                        | 203/205                         | 8/9               | 42/44           | 206/206                        | 200/201                         | 10/11             | 44/45           |
| CD 70%-straightened, .206" Rd.                                               | 208/210                        | 205/205                         | 11/11             | 47/48           | 203/204                        | 201/201                         | 11/13             | 44/47           |
| CD 70%-straightened, hardened 900° F.<br>1 hr., centerless ground, .200" Rd. | 289/290                        | 286/288                         | 12/13             | 42/44           | 285/290                        | 274/277                         | 12/13             | 43/44           |

<sup>1</sup> Chemical composition: C, .042; Mn, 1.00; P, .020; S, .010; Si, .40; Cr, 14.71; Ni, 7.66; Cu, 3.19; Al, 1.16.

<sup>2</sup> P.s.i.  $\times 1,000$ .

Aluminum analysis made on 4" sq. billet section.

Here it is to be noted that for the 70% cold-drawn wire there is had a gain in strength of about 80,000 p.s.i. as a result of the age-hardening treatment (for some 208,000-210,000 p.s.i. for the drawn material to some 289,000-290,000 for the drawn and aged material). And that with the ageing there is retained good ductility (some 12-13% elongation and some 42-44% reduction in area for the aged wire as compared to some 11% elongation and some 47-48% reduction in area for the cold drawn and straightened material).

#### Conclusion

Thus it will be seen that I provide in my invention a chromium-nickel-copper-aluminum stainless steel and a method of treating the same in which the various objects hereinbefore set forth, together with many practical advantages are successfully achieved.

The steel of my invention by reason of particular chromium-nickel-copper-aluminum composition and a particular balancing of the same, readily lends itself to cold-working and cold-forming as by upsetting, rolling, spinning and the like, to effect a certain hardening of the metal. In addition, the steel lends itself to further hardening, i.e. hardening by heat-treatment at moderate temperatures, to achieve an ageing or precipitation hardening effect.

I also provide in my invention a variety of converted forms such as bar, rod, wire, sheet, strip, special shapes, and the like, readily suited to moderate hardening as a result of the cold-working and cold-forming operations noted, as in the production of a variety of articles and products which then lend themselves to age-hardening, giving a combination of high surface hardness, abrasion-resistance and wearability, together with internal toughness and ductility.

Since many embodiments may be made of my invention and since numerous changes may be made in the embodiments hereinbefore set forth, it will be understood that all matter described herein or shown in the accompanying drawing, is to be interpreted as illustrative and not by way of limitation.

I claim as my invention:

1. A chromium-nickel-copper-aluminum stainless steel which is but moderately hardenable by cold-work and which thereafter is substantially hardenable by ageing heat-treatment, said steel consisting essentially of about 10% to 25% metal of the group consisting of chromium and molybdenum with an actual chromium content of at least 10% and molybdenum up to 5%, the molybdenum being substituted for chromium on a 1 to 1 basis; about 5% to 20% metal of the group consisting of nickel

on a 2 to 1 basis with the relation between the two groups being:

|    | Chromium-molybdenum,<br>percent: | Nickel-manganese,<br>percent |
|----|----------------------------------|------------------------------|
| 30 | 10                               | 13 to 20                     |
|    | 12                               | 8 to 20                      |
|    | 16                               | 7 to 20                      |
|    | 19                               | 6.5 to 20                    |
|    | 22                               | 5 to 20                      |
| 35 | 25                               | 5 to 20                      |

about 1% to 5% copper; about .25% to 2.50% aluminum; and remainder substantially all iron.

2. A chromium-nickel-copper-aluminum stainless steel which is but moderately hardenable by cold-work and age-hardened, which cold-worked and aged steel is essentially non-magnetic and consists essentially of about 10% to 25% metal of the group consisting of chromium and molybdenum, with an actual chromium content of at least 10% and molybdenum up to 5% as a substitute for chromium on a 1 to 1 basis; about 11% to 20% metal of the group consisting of nickel and manganese, with an actual nickel content of at least 4% and manganese up to 15% substituted for nickel on a 2 to 1 basis; about 1% to 4% copper; about .25% to 2.50% aluminum; and remainder substantially all iron.

3. A chromium-nickel-copper-aluminum stainless steel which is but moderately hardenable by cold-work and which thereafter is substantially hardened by ageing heat-treatment, said steel in the cold-worked and aged condition being substantially magnetic and consisting essentially of about 10% to 22% chromium; about 5% to 16% nickel, with the relation between the chromium and the nickel within the broad ranges being:

|    | Chromium, percent: | Nickel, percent |
|----|--------------------|-----------------|
| 60 | 10                 | 13 to 16        |
|    | 12                 | 8 to 14         |
|    | 16                 | 7 to 13         |
|    | 19                 | 6.5 to 9.5      |
| 65 | 22                 | 5 to 6          |

about 1% to 4% copper; about .25% to 2.50% aluminum; carbon not exceeding 0.10%; and remainder substantially all iron.

4. A chromium-nickel-copper-aluminum stainless steel which is but moderately hardenable by cold-work and which thereafter is substantially hardenable by ageing heat-treatment, which cold-worked and aged steel is essentially non-magnetic and consists essentially of about

10% to 25% chromium; about 11% to 20% nickel, with the relation between the two being:

| Chromium, percent: | Nickel, percent |
|--------------------|-----------------|
| 10                 | 15 to 20        |
| 12                 | 14 to 20        |
| 16                 | 12 to 20        |
| 19                 | 11 to 20        |
| 22                 | 14 to 20        |
| 25                 | 15 to 20        |

about 1% to 4% copper; about .25% to 2.5% aluminum; carbon not exceeding 0.10%; and remainder substantially all iron.

5. A chromium-nickel-copper-aluminum stainless steel which is but moderately hardenable by cold-work and which thereafter is substantially hardenable by ageing heat-treatment; said steel consisting essentially of about 14% to 19% chromium; about 7% to 13% nickel, with the nickel being at least about 8% for a chromium content of 14% and at least about 7% for a chromium content of 19%; about 1% to 5% copper; about .5% to 2% aluminum; a carbon content not exceeding 0.10%; a nitrogen content not exceeding 0.10%; and remainder substantially all iron.

6. A chromium-nickel-copper-aluminum stainless steel which is but moderately hardenable by cold-work and which thereafter is substantially hardenable by ageing heat-treatment, said steel consisting essentially of about 14% to 19% chromium; about 7% to 13% nickel, with nickel being at least about 8% for a chromium content of 14% and at least about 7% for a chromium content of 19%; about 1% to 4% copper; about .5% to 2% aluminum; with carbon and nitrogen taken together not exceeding 0.10%; and remainder substantially all iron.

7. A chromium-nickel-copper-aluminum stainless steel which is but moderately hardenable by cold-work and age-hardened, which cold-worked and aged steel is essentially non-magnetic and consists essentially of about 15% to 18% chromium; about 11% to 13% nickel; about 2% to 4% copper; about .75% to 1.50% aluminum; and remainder substantially all iron.

8. Stainless steel product cold-reduced 70% to 90% and age-hardenable to great strength and hardness with significant ductility, said product essentially consisting of about 15% to 18% chromium; about 7% to 10% nickel; about 2% to 5% copper, about .75% to 1.50% aluminum; and remainder substantially all iron.

9. Stainless steel product cold-reduced 70% to 90% and age-hardenable to great strength and hardness along with significant ductility, said product essentially consisting of about 15% to 18% chromium; about 11% to 13% nickel; about 2% to 5% copper; about .75% to 1.50% aluminum; and remainder substantially all iron.

10. Cold-formed stainless steel threaded fastener comprising a cold-reduced rolled-on threaded portion and a tough ductile core portion, said threaded portion being in age-hardened condition and the tough ductile core portion being not substantially age-hardened, said fastener consisting essentially of about 10% to 25% metal of the group chromium and molybdenum, with an actual chromium content of at least 10% and molybdenum up to 5% being substituted for chromium on a 1 to 1 basis; about 5% to 20% metal of the group nickel and manganese, with an actual nickel content of at least 4% and manganese up to 15% being substituted for nickel on a 2 to 1 basis; about 1% to 5% copper; about .25% to 2.50% aluminum; and remainder substantially all iron.

11. Cold-formed stainless steel threaded fastener which is essentially non-magnetic comprising a cold-reduced rolled-on threaded portion and a tough ductile core portion, said threaded portion being in age-hardened condition and the tough ductile core portion being not sub-

stantially age-hardened, which fastener consists essentially of about 10% to 25% metal of the group chromium and molybdenum, with an actual chromium content of at least 10% and molybdenum up to 5% as a substitute for chromium on a 1 to 1 basis; about 11% to 20% metal of the group nickel and manganese, with an actual nickel content of at least 4% and manganese up to 15% substituted for nickel on a 2 to 1 basis; about 1% to 4% copper; about .25% to 2.50% aluminum; and remainder substantially all iron.

10. Age-hardened stainless steel self-tapping drive screw comprising a rolled-on threaded portion of hard surface; and a tough ductile core portion, which screw is substantially magnetic and consists essentially of about 15% to 18% chromium; about 7% to 10% nickel; about 2% to 5% copper; about .75% to 1.50% aluminum; and remainder substantially all iron.

13. Age-hardened stainless steel self-tapping drive screw comprising a rolled-on threaded portion of hard surface; and a tough ductile core portion; which screw is essentially non-magnetic and consists essentially of about 15% to 18% chromium; about 11% to 13% nickel; about 2% to 5% copper; about .75% to 1.50% aluminum; and remainder substantially all iron.

14. Stainless steel spring cold-reduced at least 70% and subsequently age-hardened, said spring consisting essentially of about 10% to 25% metal of the group chromium and molybdenum with an actual chromium content of at least 10% and molybdenum up to 5% being substituted for chromium on a 1 to 1 basis; about 5% to 20% metal of the group nickel and manganese with an actual nickel content of at least 4% and manganese up to 15% being substituted for nickel on a 2 to 1 basis with the relation between the two groups being:

| Chromium-molybdenum, percent: | Nickel-manganese, percent: |
|-------------------------------|----------------------------|
| 10                            | 13 to 20                   |
| 12                            | 8 to 20                    |
| 16                            | 7 to 20                    |
| 19                            | 6.5 to 20                  |
| 22                            | 5 to 20                    |
| 25                            | 5 to 20                    |

about 1% to 5% copper; about .25% to 2.50% aluminum; and remainder substantially all iron.

15. Magnetic stainless steel spring essentially consisting of about 15% to 18% chromium; 7% to 10% nickel; about 2% to 5% copper; about .75% to 1.50% aluminum; and remainder substantially all iron.

16. Non-magnetic stainless steel spring essentially consisting of about 15% to 18% chromium; about 11% to 13% nickel; about 2% to 5% copper; about .75% to 1.50% aluminum; and remainder substantially all iron.

17. Radio antenna wire essentially consisting of about 15% chromium, about 8% nickel, about 3% copper, about 1% aluminum, and remainder substantially all iron.

#### References Cited

#### UNITED STATES PATENTS

|    |           |         |             |            |
|----|-----------|---------|-------------|------------|
| 60 | 2,505,763 | 5/1950  | Goller      | 75—124     |
|    | 2,553,706 | 5/1951  | Goller      | 148—121.3X |
|    | 2,553,707 | 5/1951  | Goller      | 148—12.3X  |
|    | 2,614,921 | 10/1952 | Tanczyn     | 75—124     |
| 65 | 2,694,626 | 11/1954 | Tanczyn     | 75—124     |
|    | 3,069,961 | 12/1962 | Baubles     | 10—152     |
|    | 3,152,934 | 10/1964 | Lula et al. | 75—124     |

HYLAND BIZOT, Primary Examiner.

DAVID L. RECK, Examiner.

P. WEINSTEIN, Assistant Examiner.